

**United States Patent** [19]

Taniguchi et al.

[11] **Patent Number:** **4,970,131**[45] **Date of Patent:** **Nov. 13, 1990**[54] **ELECTROPHOTOGRAPHIC  
PHOTOCONDUCTOR HAVING OVERCOAT  
LAYER**[75] Inventors: **Kiyoshi Taniguchi; Toshio Fukagai;  
Kayoko Yokoyama**, all of Numazu,  
Japan[73] Assignee: **Ricoh Company, Ltd.**, Tokyo, Japan[21] Appl. No.: **395,091**[22] Filed: **Aug. 16, 1989**[30] **Foreign Application Priority Data**

Aug. 29, 1988 [JP] Japan ..... 63-214553

Aug. 29, 1988 [JP] Japan ..... 63-214555

Sep. 16, 1988 [JP] Japan ..... 63-231783

Sep. 16, 1988 [JP] Japan ..... 63-231784

[51] Int. Cl.<sup>5</sup> ..... **G03G 5/14**[52] U.S. Cl. ..... **430/67; 430/66**[58] Field of Search ..... **430/66, 67**[56] **References Cited****U.S. PATENT DOCUMENTS**

4,006,020 2/1977 Polastri ..... 430/67

*Primary Examiner*—J. David Welsh*Attorney, Agent, or Firm*—Oblon, Spivak, McClelland,  
Maier & Neustadt[57] **ABSTRACT**

An electrophotographic photoconductor is disclosed, which comprises an electroconductive support, a photoconductive layer formed on the electroconductive support, and an overcoat layer formed on the photoconductive layer, in which the overcoat layer comprises a binder resin and one component selected from the group consisting of a crown ether, a polyalkylene glycol, a polyalkylene glycol ester and a polyalkylene glycol ether. The overcoat layer may be composed of an intermediate layer formed on the photoconductive layer, and a protective layer formed on the intermediate layer in such a manner that any of the crown ether and polyalkylene glycol derivatives is contained in the intermediate layer.

**45 Claims, No Drawings**

**ELECTROPHOTOGRAPHIC  
PHOTOCONDUCTOR HAVING OVERCOAT  
LAYER**

**BACKGROUND OF THE INVENTION**

1. Field of the Invention

This invention relates to an improved electrophotographic photoconductor.

2. Discussion of Background

Recently, organic photoconductive materials, which are relatively inexpensive and cause no environmental pollution, have been widely used as photoconductors of electrophotographic copying machines.

As an organic electrophotographic photoconductor, there have been known photoconductive resin type photoconductors, typically a photoconductor comprising polyvinyl carbazole (PVK), charge-transport complex type photoconductors, typically a photoconductor comprising polyvinyl carbazole 2,4,7-trinitro-fluorenone (PVK-TNF), pigment-dispersed type photoconductors, typically a photoconductor in which phthalocyanine is dispersed in a binder resin, and function-separated type photoconductors such as a photoconductor consisting essentially of a charge-generating material and a charge-transporting material. Of these, the last one is currently attracting much attention.

When a high-photosensitive photoconductor of the function-separate type is applied to the Carlson process, it exhibits low chargeability and weak electric charge retention (large dark decay). Furthermore, the chargeability and electric charge retention properties are drastically deteriorated in the course of repeated and continuous use, causing uneven image density and fogging. In addition, toner particles are unfavorably deposited on the background when reverse development is performed.

In general, the chargeability of the high photo-sensitive photoconductor is reduced due to pre-exposure fatigue. Such fatigue is chiefly caused by the light absorbed by the charge-generating material contained in the photoconductor. It is therefore considered that the longer the period in which the electric charges generated by the light absorption remain in a migrational state in the photoconductor and the greater the number of the generated electric charges, the greater the reduction in the chargeability of the photoconductor. Even if the photoconductor is electrically charged while the electric charges generated by light-absorption are in a residual state, the surface potential will not be elevated until the residual electric charges are dissipated. This is because the electric charges at the surface of the photoconductor are neutralized with the residual carriers which migrate in the photoconductor. The rise of surface potential is thus delayed corresponding to the pre-exposure fatigue, so that the apparent surface potential is lowered.

In an attempt to overcome the above shortcomings in the prior art, the following protective layers have been proposed: a protective layer in which aluminous fibers are dispersed as disclosed in Japanese Laid-Open Pat. Application 55-45024; protective layers in which  $Al_2O_3$ ,  $SiO_2$ ,  $SiC$ ,  $SiO_2$ ,  $Al_2O_3$  and  $B4C$  are each dispersed as disclosed in Japanese Laid-Open Pat. Applications 56-38054, 56-99347 and 57-165848; a protective layer in which  $SnO_2$  and  $Sb_2O_3$  are dispersed as disclosed in Japanese Laid-Open Pat. Application 58-121044; a protective layer in which  $CuI$  is dispersed

as disclosed in Japanese Laid-Open Pat. Application 59-159; a protective layer in which  $TiO_2$  is dispersed as disclosed in Japanese Laid-Open Pat. Application 60-75842; protective layers in which indium oxide is

5 dispersed as disclosed in Japanese Laid-Open Pat. Applications 57-30846 and 57-154250; and a protective layer coated with  $MgF_2$ ,  $SiN_4$ ,  $Al_2O_3$  or  $ZrO_2$  by means of sputtering as disclosed in Japanese Laid-Open Pat. Application 58-59459.

10 Furthermore, the following intermediate layers have also been proposed: an intermediate layer in which an organic titanium compound is dispersed as disclosed in Japanese Laid-Open Pat. Application 58-18637; intermediate layers in which organic metallic compounds are dispersed as disclosed in Japanese Laid-Open Pat. Applications 58-60748 and 59-46653; an intermediate layer in which zirconium alkoxide or zirconium alkoxide with a silane coupling agent is dispersed as each disclosed in Japanese Laid-Open Pat. Applications 59-223438 and 58-121043; intermediate layers in which thermoplastic polycarbonate resin, acrylate resin and methacrylate resin are each dispersed as disclosed in Japanese Laid-Open Pat. Applications 60-12552, 20 60-142341 and 60-117561.

15 The above-mentioned protective layers and intermediate layers, however, cannot sufficiently prevent the reduction in chargeability caused by the repeated and continuous use of the photoconductors, the delay in the rise of the surface potential thereof, or the considerable change in the residual electric potential.

**SUMMARY OF THE INVENTION**

It is therefore an object of the present invention to provide an improved electrophotographic photoconductor which is highly sensitive, shows extremely small reduction in the chargeability caused by pre-exposure fatigue, and exhibits no delay in the rise of the charged potential and minimal changes in the residual electric potential even after extended periods of repeated charging and exposing.

The foregoing object of the present invention can be attained by an electrophotographic photoconductor comprising an electroconductive support, a photoconductive layer formed on the electroconductive support, and an overcoat layer formed on the photoconductive layer, wherein the overcoat layer comprises a binder resin and one component selected from the group consisting of a crown ether, a polyalkylene glycol, a polyalkylene glycol ester, and a polyalkylene glycol ether.

**DETAILED DESCRIPTION OF THE  
PREFERRED EMBODIMENTS**

In the present invention, the overcoat layer, which is a single layer and serves as a protective layer, is formed on the photoconductive layer, and a crown ether, polyalkylene glycol, polyalkylene glycol ester or polyalkylene glycol ether is incorporated therein.

The overcoat layer can also be made of two layers which are an intermediate layer formed on the electroconductive support and a protective layer formed on the intermediate layer. In this case, one of the above crown ether and polyalkylene derivatives is incorporated into the intermediate layer.

Thus, the electrophotographic photoconductor of the present invention comprises a crown ether, polyalkylene glycol, polyalkylene glycol ester or polyalkylene glycol ether in the overcoat layer or the interme-

ate layer, so that the degree of reduction in the chargeability after repeated and continuous use, the delay in the rise of the surface potential and the change in the residual electric potential can be effectively minimized. 5

In the present invention, it is preferably to employ a crown ether containing 3 to 8 oxygen atoms in its ring. Examples of such crown ethers are as follows:



12-crown-4-ether,



18-crown-6-ether,



dibenzo-18-crown-6-ether



tribenzo-18-crown-6-ether,



dicyclohexano-18-crown-6-ether,

-continued



tetrabenzo-24-crown-8-ether,



15-crown-5-ether



21-crown-7-ether



benzo-15-crown-5-ether,



dibenzo-24-crown-8-ether,

-continued



dicyclohexano-24-crown-8-ether,



poly(dibenzo-18-crown-6-ether), and



a crown ether having the following formula



When the crown ether is incorporated into the overcoat layer, it is used in an amount of 0.01 to 10 parts by weight, preferably 0.1 to 1 parts by weight, per 1 part by weight of the binder resin contained in the overcoat layer. When the crown ether is incorporated into the intermediate layer, it is used in an amount of 0.1 to 50 parts by weight, preferably 0.2 to 20 parts by weight, per 100 parts by weight of the binder resin contained in the intermediate layer.

Examples of the polyalkylene glycols used in the present invention include polyethylene glycols, polypropylene glycols, polybutylene glycols, and random copolymers and block copolymers of hydroxyethylene and hydroxypropylene. Commercially available polyalkylene glycols of the above types can be used in the present invention.

Regarding the polyethylene glycols, those having a molecular weight ranging from 100 to 5,000,000, preferably from 200 to 50,000, are employed in the present invention. (Those having a molecular weight of 10,000 or more may be referred to as polyethylene oxide.)

With respect to the polypropylene glycols, those having a molecular weight ranging from 130 to 500,000, preferably from 500 to 10,000, are employed.

In the case of the polybutylene glycols, those having a molecular weight ranging from 160 to 100,000, preferably from 500 to 3,000, are employed.

Regarding the random and block copolymers of hydroxyethylene and hydroxypropylene, those having a molecular weight ranging from 200 to 500,000, preferably from 500 to 50,000, and a mean number of added moles of an oxyethylene group of 0.1 to 99.9 mol% are employed.

Specific examples of the polyalkylene glycols which are preferably employed in the present invention include polyethylene glycol monocarboxylic acid esters, polyethylene glycol dicarboxylic acid esters, and carboxylic acid esters of polyoxyethylene sorbitan.

Examples of the commercially available polyethylene glycol monocarboxylic acid esters usable in the present invention are as follows:

“Ionet MS-400”, “Ionet MS-1000”, “Ionet MO-200”, “Ionet MO-400”, “Ionet MO-600” and “Santopearl TE-106” (Trademarks), all available from Sanyo Chemical Industries, Ltd.;

25 “Noigen ES” (Trademark) series, available from Dai-Ichi Kogyo Seiyaku Co., Ltd.; and

“Nonion L” (Trademark) series, “Nonion S” (Trademark) series, “Nonion O” (Trademark) series and “Nonion T” (Trademark) series, all available from Nippon Oil & Fats Co., Ltd.

Examples of the commercially available polyethylene glycol dicarboxylic acid esters usable in the present invention are as follows:

35 “Ionet DL-200”, “Ionet DS-300”, “Ionet DS-400”, “Ionet DO-200”, “Ionet DO-400”, “Ionet DO-600”, “Ionet DO-1000” and “Santopearl GE-70” (Trademarks), all available from Sanyo Chemical Industries, Ltd.; and

40 “Nonion DS-60HN” (Trademark) (distearate), available from Nippon Oil & Fats Co., Ltd.

Examples of the commercially available carboxylic acid esters of polyethylene sorbitan usable in the present invention are as follows:

45 “Tween” (Trademark), available from Atlas Powder Corp.;

“Ionet T-20C”, “Ionet T-60C” and “Ionet T-80C” (Trademarks), all available from Sanyo Chemical Industries, Ltd.;

50 “Adeka Estol T-62” and “Adeka Estol T-82” (Trademarks), both available from Asahi Denka Kogyo K.K.;

“Sorgen TW” (Trademark) series, available from Dai-Ichi Kogyo Seiyaku Co., Ltd.; and

“Nonion LT-221”, “Nonion PT-221”, “Nonion ST-221” and “Nonion OT-221” (Trademarks), all available from Nippon Oil & Fats Co., Ltd.

Specific examples of the polyalkylene glycol ethers used in the present invention include polyethylene glycol monoethers, polypropylene glycol monoethers and monoethers of copolymers of hydroxyethylene and hydroxypropylene. Commercially available polyalkylene glycol monoethers of the above type can be employed in the present invention.

The polyethylene glycol monoether is represented by 65 the following formula:



wherein R represents an alkyl group having 1 to 30 carbon atoms, preferably 10 to 20 carbon atoms, a substituted or unsubstituted aryl group, or most preferably a phenyl group substituted with an alkyl group having 1 to 20 carbon atoms, and n represents the mean number of added moles of a hydroxyethylene group, which is an integer of 1 or more, preferably 2 to 1000.

Examples of commercially available polyethylene glycol monoethers having the above formula are as follows:

"Emulmin 40", "Emulmin 50", "Emulmin 60", "Emulmin 70", "Emulmin 110", "Emulmin 140", "Emulmin 180", "Emulmin M-20", "Emulmin 240", "Emulmin L-90-S", "Emulmin L-380", "Nonipol 20", "Nonipol 30", "Nonipol 40", "Nonipol 55", "Nonipol 60", "Nonipol 70", "Nonipol 85", "Nonipol 91", "Nonipol 95", "Nonipol 100", "Nonipol 110", "Nonipol 120", "Nonipol 130", "Nonipol 140", "Nonipol 160", "Nonipol 200", "Nonipol 290", "Nonipol 300", "Nonipol 400", "Nonipol 450", "Nonipol 500", "Nonipol 700", "Nonipol 800", "Nonipol D160", "Octapol 45", "Octapol 50", "Octapol 60", "Octapol 80", "Octapol 100", "Octapol 200", "Octapol 300", "Octapol 400", "Dodecapol 61", "Dodecapol 90", "Dodecapol 120" and "Dodecapol 200" (Trademarks), all available from Sanyo Chemical Industries, Ltd.;

"Adeka Estol OEG" (Trademark) series and "Adeka Estol SEG" (Trademark) series, all available from Asahi Denka Kogyo K.K.;

"Noigen ET" (Trademark) series, "Noigen EA" (Trademark) series, "Emulsit L" (Trademark) series, and "Emulsit" (Trademark) series, all available from Dai-Ichi Kogyo Seiyaku Co., Ltd.; and

"Nonion E-206", "Nonion E-215", "Nonion E-230", "Nonion P-208", "Nonion P-210", "Nonion P-213", "Nonion S-207", "Nonion S-215", "Nonion S-220", "Nonion K-204", "Nonion K-215", "Nonion K-220", "Nonion K-230", "Nonion T-2085", "Nonion NS" series, "Nonion HS" series, "Persoft NK-60", "Persoft NK-100", "Uniox M-400", "Uniox M-550", "Uniox M-200" and "Uniox C-2300" (Trademarks), all available from Nippon Oils & Fats Co., Ltd.

The polypropylene glycol monoether is represented by the following formula:



wherein R represents an alkyl group having 1 to 30 carbon atoms, preferably 10 to 20 carbon atoms, a substituted or unsubstituted aryl group, or most preferably a phenyl group substituted with an alkyl group having 1 to 20 carbon atoms, and n represents the mean number of added moles of a hydroxypropylene group, which is an integer of 1 or more, preferably 5 to 100.

Examples of commercially available polypropylene glycol monoether having the above formula include the products of Sanyo Chemical Industries, Ltd. with the trademarks of "Newpol LB-65", "Newpol LB-285", "Newpol LB-385", "Newpol LB-125", "Newpol LB-1145", "Newpol LB-1715", "Newpol LB-3000", "Newpol LB-300X", "Newpol LB-400XY", "Newpol LB-650X" and "Newpol LB-1800X".

Monoethers of a copolymer of hydroxyethylene and hydroxypropylene are known compounds, and commercially available products of the monoethers having a molecular weight of 200 to 20,000, more preferably 200 to 4,000, can be employed in the present invention.

Specific examples of such monoethers include the products of Sanyo Chemical Industries, Ltd. with the

trademarks of "Newpol 50HB-55", "Newpol 50HB-100", "Newpol 50HB-260", "Newpol 50HB-400", "Newpol 50HB-660", "Newpol 50HB-2000" and "Newpol 50HB-5100".

When the above-described polyalkylene glycol, polyalkylene glycol ester or polyalkylene glycol ether is incorporated into the overcoat layer, it is used in an amount of 0.01 to 10 parts by weight, preferably 0.1 to 1 parts by weight, per 1 part by weight of the binder resin contained in the overcoat layer. When one of these compound is incorporated into the intermediate layer, it is used in an amount of 0.1 to 50 parts by weight, preferably 0.2 to 20 parts by weight, per 100 parts by weight of the binder resin contained in the intermediate layer.

The overcoat layer and the photoconductive layer are formed in the same manner. The preferred thickness of the overcoat layer is 1 to 30  $\mu m$ . Furthermore, it is preferable to incorporate finely-divided particles of a metallic oxide such as  $SnO_2$ ,  $Sb_2O_3$ ,  $In_2O_3$  and  $TiO_2$  into the overcoat layer in order to prevent the rise of the residual electric potential. The amount of the metallic oxide is 10 to 80 wt. % of the entire weight of the overcoat layer. The particle size of the metallic oxide is 0.5  $\mu m$  or less, preferably 0.3  $\mu m$  or less.

In the case where the overcoat layer is composed of the intermediate layer and the protective layer, the intermediate layer has a thickness of 10  $\mu m$  or less, preferably 1  $\mu m$  or less, and the protective layer has a thickness ranging from 1 to 30  $\mu m$ .

Into this protective layer, it is preferable to incorporate finely-divided particles of a metallic oxide which are the same as those employed in the overcoat layer.

For the binders in the overcoat layer and the intermediate layer, the following thermoplastic and thermosetting resins can be employed; for example, polystyrene, a copolymer of styrene and acrylonitrile, a copolymer of styrene and butadiene, a copolymer of styrene and maleic anhydride, polyester, polyvinyl chloride, a copolymer of vinyl chloride and vinyl acetate, polyvinyl acetate, polyethylene, polypropylene, polyvinylidene chloride, fluorine-contained resin, polyacrylate resin, phenoxy resin, polycarbonate, polyamide, cellulose acetate resin, ethyl cellulose resin, polyvinyl butyral, polyvinyl formal, polyvinyl toluene, poly-N-vinyl carbazole, acrylic resin, silicone resin, epoxy resin, melamine resin, urethane resin, phenol resin, alkyd resin and cellulose.

The present invention will now be explained in more detail.

In the present invention, the conductive substrate is employed so as to attract electric charges of a reverse polarity from the charges generated by electrification. The materials which can be employed as the substrate are those having an electric resistance of  $10^8 \Omega$  or less, and capable of withstanding the conditions for forming the intermediate, charge generation and charge transport layers.

Examples of such materials include electroconductive metals such as Al, Ni, Cr, Zn and stainless steel, and inorganic insulation materials, such as glass and ceramics, and organic insulation materials, such as polyester, polyimide, phenol resin, nylon resin and paper. In the case of the insulating materials, their surfaces are coated with an electroconductive material, such as Al, Ni, Cr, Zn, stainless steel, carbon,  $SnO_2$  and  $In_2O_3$ , by means of vacuum deposition, sputtering or spray coating.

Either a mono-layered or a multi-layered (laminated type) photoconductive layer can be employed in the present invention.

The mono-layered photoconductive layer can serve as both a charge generation layer and a charge transport layer. When such a layer is exposed to light, latent electrostatic images are formed thereon.

In order to form the photoconductive layer of the mono-layered type, photoconductive powder such as zinc oxide, titanium oxide or sensitized zinc oxide, amorphous silicone powder, crystalline selenium powder, a phthalocyanine pigment, or an azo pigment is coated onto the electroconductive substrate together with a binder resin and, if necessary, charge transporting materials which will be described later. Binder resins which are employed in the multi-layered photoconductor can be employed in the above layer. Such binder resins will be described later.

Furthermore, a mono-layered photoconductive layer which is made of the charge transporting material and a eutectic crystalline complex prepared by a pyrylium dye and a bisphenol A type polycarbonate can also be employed in the present invention.

It is preferable that the mono-layered photoconductive layer have a thickness ranging from 5 to 30  $\mu\text{m}$ .

The laminated type photoconductive layer consists of a charge generation layer and a charge transport layer. The charge transport layer transports the charges which are generated in and liberated from the charge generation layer under the application of light. It also dissipates the charges which are induced in the electroconductive layer. The charge transport layer is required to have high electric resistance so that the electric charges can be maintained. It is also required to have low dielectric constant and high charge transportation ability so that high surface potential can be obtained by the electric charges maintained. In order to meet the above requirements, an organic charge transport layer containing as an effective component an organic charge transporting material is employed.

Generally known compounds can be employed as the organic charge transporting material, such as poly-N-vinyl carbazole compounds, pyrazoline compounds,  $\alpha$ -phenylstilbene compounds, hydrazone compounds, diarylmethane compounds, triphenyl amine com-

pounds, divinyl benzene compounds, fluorene compounds, anthracene compounds, oxadiazole compounds, and diamino carbazole compounds.

When the above organic charge transporting materials other than the polymers such as polyvinyl carbazole compounds are employed, they are, in advance, incorporated into a polymer or copolymer resin such as polyamide resin, polyurethane resin, polyester resin, epoxy resin, poly-carbonate resin, polyether resin (all polycondensed type), polystyrene resin, polyacrylate resin, polymethacrylate resin, poly-N-vinyl carbazole resin, polyvinyl butyral resin, a styrene—butadiene copolymer resin, and a styrene-acrylonitrile copolymer resin.

A plasticizer may be incorporated into the above mixture of the organic charge transporting material and the resin, if necessary. Examples of the plasticizer include halogenated paraffin, dimethyl naphtharene, diethyl phthalate, dioctylphthalate, tricresyl phosphate, and polymers and copolymers such as polyester.

The charge transporting material, the binder resin and silicone oil which serves as a labelling agent are dissolved in a proper organic solvent. The resulting solution is coated onto the electroconductive substrate by means of roller coating, dip coating, spray coating or blade coating, and dried at a temperature between 50 and 200° C. Thus, an electric charge transport layer having a thickness between 5 and 100  $\mu\text{m}$  can be obtained.

The weight ratio of the charge transporting material to the binder resin is 2:8 to 8:2; and the incorporated amount of the silicone oil is 0.001 to 1 parts by weight per 100 parts by weight of the binder resin.

The charge generation layer generates electric charges when the layer is exposed to light, and liberates them from the layer. In the present invention, the charge generation layer contains as a charge generating material an organic dye, an organic pigment, crystalline selenium, or arsenic selenide.

Examples of the organic dye and pigment include phthalocyanine pigments, disazo pigments, trisazo pigments, perylene pigments, squalic salt dyes, azulenium salt dyes, and quinone condensed multi-ring compounds.

Specific examples of the disazo pigment and the trisazo pigments are as follows.

Pigment No.

A



1



-continued

Pigment No.

A

2



3



4



5



6



-continued

Pigment No.

A

7



8



9



10



11



-continued

| Pigment No. | A |
|-------------|---|
| 12          |   |
| 13          |   |
| 14          |   |
| 15          |   |

-continued

Pigment No.

A

16



17



18



19



20



-continued

Pigment No.

A

21



22



23



24



-continued

Pigment No.

A

25



26



27



28



29



-continued

| Pigment No. | A                                                                                   |
|-------------|-------------------------------------------------------------------------------------|
| 30          |    |
| 31          |    |
| 32          |   |
| 33          |  |
| 34          |  |

-continued

Pigment No.

A

35



36



37



38



-continued

Pigment No.

A

39



40



41



42



-continued

Pigment No.

A

43



44



45



46



-continued

Pigment No.

A

47



48



49



50



-continued

Pigment No.

A

51



52



53



54



55



-continued

| Pigment No. | A                                                                                   |
|-------------|-------------------------------------------------------------------------------------|
| 56          |    |
| 57          |    |
| 58          |   |
| 59          |  |
| 60          |  |

-continued

Pigment No.

A

61



62



63



64



65



-continued

Pigment No.

A

66



67



68



69



-continued

Pigment No.

A

70



71



72



73



74



These organic dyes and pigments are dispersed in an organic solvent with or without a resin in a ball mill, a sand mill, a kneader having three rollers, an attriter, or a dispersing apparatus using ultrasonic wave.

As the binder resin which is used together with the above organic dyes or pigments, the same resins as used in the charge transport layer can be employed.

The charge generation layer can be formed in the same manner as in the formation of the charge transport layer. The preferred thickness of the charge generation layer is in the range of 0.05 to 10  $\mu\text{m}$ .

In the case where crystalline selenium or arsenic selenide powder is used as the charge generating material in the charge generation layer, a charge transporting binder agent and/or a charge transporting organic compound is co-employed.

55

Examples of such charge transporting materials include polyvinyl carbazole and its derivatives such as those having a substituent of a halogen such as chlorine or bromine, a methyl group or an amino group in its carbazole structure, polyvinyl pyrene, oxadiazole, pyrazoline, hydrazone, diarylmethane,  $\alpha$ -phenylstilbene, diaryl methane compounds, and nitrogen-containing compounds such as triphenyl amine. Of these compounds, polyvinyl carbazole and derivatives thereof are preferably employed in the present invention.

60

The above compounds can be employed either singly or in combination. In the case where they are employed in combination, the use of polyvinyl carbazole or derivatives thereof and other above-mentioned charge transporting compounds is preferable.

65

In order to improve adhesion and plasticity, binder resins which are used with the organic dyes and pigments can also be employed with the crystalline selenium or arsenic selenide powder.

The amount of the charge generating material is preferably 30 to 90 wt.% of the entire weight of the charge generation layer, and the thickness of the charge generation layer is preferably 0.2 to 5  $\mu\text{m}$ .

Other features of this invention will become apparent in the course of the following description of exemplary embodiments, which are given for illustration of the invention and are not intended to be limiting thereof.

#### Example 1-1

##### Preparation of Charge Transport Layer Forming Liquid

A charge transport layer forming liquid No. 1-1 having the following formulation was prepared.

|                                                                                      | parts by weight |
|--------------------------------------------------------------------------------------|-----------------|
| $\alpha$ -Phenylstilbene having the following formula (charge transporting material) | 10              |
|    |                 |
| Polycarbonate (Trademark "Panlite C-1400" made by Teijin Limited)                    | 10              |
| Silicone oil (Trademark "KF50", made by Shin-Etsu Silicone Co., Ltd.)                | 0.0002          |
| Tetrahydrofuran                                                                      | 80              |

##### Preparation of Charge Generation Layer Forming Liquid

The previously mentioned azo pigment No. 1 and cyclohexanone in a weight ratio of 1:16 were placed in a ball mill pot, followed by ball-milling for 48 hours by using stainless steel balls.

Thereafter, the same amount of cyclohexanone was added to the above mixture, and ball-milling was continued for a further 24 hours.

The resulting mixture taken out of the ball mill was diluted with cyclohexanone under stirring whereby a charge generation layer forming liquid No. 1-1 was obtained, which contained 1 wt.% of the solid components.

##### Preparation of Overcoat Layer Forming Liquid

A mixed resin consisting of 20 wt.% styrene, 30 wt.% methylmethacrylate, 25 wt.% acrylic acid and 25 wt.% N-methyrol acrylamide was dissolved in a 9:1 mixed solvent of toluene and butanol so that the resulting solution contained 40 wt.% of the mixed resin. 30 parts by weight of the solution thus prepared and 12 parts by weight of  $\text{SnO}_2$  powder were dispersed in a suitable amount of a 9:1 mixed solvent of toluene and n-butanol

in a ball mill for 72 hours. To the resulting dispersion, 3 parts by weight of dibenzo-18-crown-6-ether was added, and stirred, whereby an overcoat layer forming liquid No. 1-1 was obtained.

##### Preparation of Photoconductor

An aluminum substrate was dip-coated with the above-prepared charge transport layer forming liquid at a pulling up speed of 6 mm/sec, and dried at 120° C. for 30 minutes, thereby forming a charge transport layer 20  $\mu\text{m}$  in thickness on the substrate.

Thereafter, the charge generation layer forming liquid was dip-coated onto the charge transport layer at a pulling up speed of 5 mm/sec, and dried at 120° C. for 20 minutes, thereby forming a charge generation layer on the charge transport layer.

Finally, the overcoat layer forming liquid was spray-coated onto the above charge generation layer, and heated at 130° C. for 30 minutes, thereby forming an overcoat layer 5  $\mu\text{m}$  in thickness on the charge generation layer.

Thus, a photoconductor No. 1-1 according to the present invention was prepared.

##### COMPARATIVE EXAMPLE 1-1

Example 1-1 was repeated except that dibenzo-18-crown-6-ether was eliminated from the overcoat layer forming liquid prepared in Example 1-1, whereby a comparative photoconductor No. 1-1 was prepared.

##### EXAMPLE 1-2

Example 1-1 was repeated except that the azo pigment No. 1 used in the charge generation layer forming liquid No. 1-1 was replaced with the azo pigment No. 47, whereby a photoconductor No. 1-2 according to the present invention was prepared.

##### EXAMPLE 1-3

Example 1-1 was repeated except that dibenzo-18-crown-6-ether used in the overcoat layer forming liquid No. 1-1 was replaced with 18-crown-6-ether, whereby a photoconductor No. 1-3 according to the present invention was prepared.

##### EXAMPLE 1-4

Example 1-1 was repeated except that an intermediate layer having a thickness of 0.1  $\mu\text{m}$  was interposed between the charge generation layer and the overcoat layer, whereby a photoconductor No. 1-4 according to the present invention was prepared.

The intermediate layer was formed in the following manner. An intermediate layer forming liquid consisting of 2 parts by weight of nylon resin (Trademark "CM 8000" made by Toray Industries, Inc.), 60 parts by weight of methanol and 38 parts by weight of butanol was dip-coated onto the charge generation layer at a pulling up speed of 3 mm/sec, and dried at 120° C. for 20 minutes

##### EXAMPLE 1-5

Example 1-1 was repeated except that the overcoat layer forming liquid No. 1-1 was replaced with the following overcoat layer forming liquid No. 1-5, whereby a photoconductor No. 1-5 according to the present invention was prepared.

## Preparation of Overcoat Layer Forming Liquid

The following components were well dispersed in a ball mill for 72 hours, and the resulting dispersion was diluted with cyclohexanone to obtain a dispersion containing 10 wt.% of the solid components.

To the above dispersion, 5 parts by weight of dibenzo-18-crown-6-ether was added, and stirred, thereby obtaining an overcoat layer forming liquid No. 1-5.

| parts by weight                                                                            |    |  |
|--------------------------------------------------------------------------------------------|----|--|
| 20% Cyclohexanone solution of phenoxy resin "PKHJ" (Trademark) made by Union Carbide Corp. | 25 |  |
| Tin oxide powder                                                                           | 5  |  |
| Cyclohexanone                                                                              | 70 |  |

## COMPARATIVE EXAMPLE 1-2

Example 1-4 was repeated except that dibenzo-18-crown-6-ether was eliminated from the overcoat layer forming liquid prepared in Example 1-4, whereby a comparative photoconductor No. 1-2 was prepared.

Each of the above electrophotographic photoconductors was positively charged in the dark under application of +6 kV of corona charge for 20 seconds. The surface potential of the photoconductor  $V_2$ , 2 seconds after the initiation of the charging, was measured by the paper analyzer. The photoconductor was then allowed to stand in the dark without applying any charge thereto until its surface potential reached +800 V. The photoconductor was then illuminated by a tungsten lamp in such a manner that the illuminance on the illuminated surface of the photoconductor was 4.5 lux so that the exposure S (lux-sec) required to reduce the surface potential (+800 V) to +400 V was measured.

The photoconductor was then exposed to a tungsten light having a color temperature of 2856° K with an exposure of 100,000 lux-sec, and the surface potential  $V_2'$  and the exposure S' were measured again in the same manner as mentioned above.

The results are shown in Table 1-1.

TABLE 1-1

| Photo-conductor | Before Fatigue |               | After Fatigue |                |
|-----------------|----------------|---------------|---------------|----------------|
|                 | $V_2$ (V)      | S (lux · sec) | $V_2'$ (V)    | S' (lux · sec) |
| No. 1-1         | 880            | 0.56          | 862           | 0.48           |
| No. 1-2         | 850            | 0.40          | 810           | 0.39           |
| No. 1-3         | 873            | 0.54          | 855           | 0.55           |
| No. 1-4         | 821            | 0.53          | 805           | 0.50           |
| No. 1-5         | 830            | 0.55          | 815           | 0.53           |
| Comp.           | 872            | 0.55          | 615           | 0.50           |
| No. 1-1         | 779            | 0.49          | 393           | 0.43           |
| No. 1-2         |                |               |               |                |

The photoconductor was attached to the surface of an Al drum having a thickness of 3 mm and a size of 80φ×340 mm. This was placed in a copying machine (Trademark "FT 4060" made by Ricoh Company Ltd.), and images were repeatedly printed. The images were usually observed at the outset of printing and after 10,000 prints had been made. The results are shown in Table 1-2.

TABLE 1-2

| Photo-conductor | Printed Images at Outset of Printing | Printed Images after 10,000-time Printing |
|-----------------|--------------------------------------|-------------------------------------------|
| No. 1-1         | clear                                | clear                                     |

TABLE 1-2-continued

| Photo-conductor | Printed Images at Outset of Printing | Printed Images after 10,000-time Printing |
|-----------------|--------------------------------------|-------------------------------------------|
| No. 1-2         | clear                                | clear                                     |
| No. 1-3         | clear                                | clear                                     |
| No. 1-4         | clear                                | clear                                     |
| No. 1-5         | clear                                | clear                                     |
| Comp.           | clear                                | Image density was found low               |
| No. 1-1         |                                      | Image density was found low               |
| Comp.           | clear                                | Image density was found low               |
| No. 1-2         |                                      | Image density was found low               |

The results of the above tests demonstrate that the electrophotographic photoconductors according to the present invention, which comprise an overcoat layer containing the crown ether, have high sensitivity, and show extremely small reduction in the chargeability caused by pre-exposure fatigue. Furthermore, the photoconductors of the present invention bring about no delay in the rise of the charged potential and a minimized change in the residual electric potential even after repeated charging and exposing.

## EXAMPLE 2-1

## Preparation of Charge Transport Layer Forming Liquid

A charge transport layer forming liquid No. 2-1 having the following formulation was prepared.

| parts by weight                                                                      |        |
|--------------------------------------------------------------------------------------|--------|
| $\alpha$ -Phenylstilbene having the following formula (charge transporting material) | 10     |
|                                                                                      |        |
| Polycarbonate (Trademark "Panlite C-1400" made by Teijin Limited)                    | 10     |
| Silicone oil (Trademark "KF50", made by Shin-Etsu Silicone Co., Ltd.)                | 0.0002 |
| Tetrahydrofuran                                                                      | 80     |

## Preparation of Charge Generation Layer Forming Liquid

The azo pigment No. 1 and cyclohexanone in a weight ration of 1:16 were placed in a ball mill pot, followed by ball-milling for 48 hours by using stainless steel balls.

Thereafter, the same amount of cyclohexanone was added to the above mixture, and ball-milling was continued for a further 24 hours.

The resulting mixture taken out of the ball mill was diluted with cyclohexanone under stirring, whereby a charge generation layer forming liquid No. 2-1 was

obtained, which contained 1 wt.% of the solid components.

#### Preparation of Overcoat Layer Forming Liquid

A mixed resin consisting of 20 wt.% styrene, 30 wt.% methylmethacrylate, 25 wt.% acrylic acid and 25 wt.% N-methyrol acrylamide was dissolved in a 9:1 mixed solvent of toluene and butanol so that the resulting solution contained 40 wt.% of the mixed resin. 30 parts by weight of the solution thus prepared and 12 parts by weight of SnO<sub>2</sub> powder were dispersed in a suitable amount of a 9:1 mixed solvent of toluene and n-butanol in a ball mill for 72 hours. To the resulting dispersion, 3 parts by weight of polyethylene glycol (Trademark "PEG6000S" made by Sanyo Chemical Industries, Ltd.) was added, and stirred, whereby an overcoat layer forming liquid No. 2-1 was obtained.

#### Preparation of Photoconductor

An aluminum substrate was dip-coated with the above-prepared charge transport layer forming liquid at a pulling up speed of 6 mm/sec, and dried at 120° C. for 30 minutes, thereby forming a charge transport layer 20  $\mu\text{m}$  in thickness on the substrate.

Thereafter, the charge generation layer forming liquid was dip-coated onto the charge transport layer at a pulling up speed of 5 mm/sec, and dried at 120° C. for 20 minutes, thereby forming a charge generation layer on the charge transport layer.

Finally, the overcoat layer forming liquid was spray-coated onto the above charge generation layer, and heated at 130° C. for 30 minutes, thereby forming a protective layer 5  $\mu\text{m}$  in thickness on the charge generation layer.

Thus, a photoconductor No. 2-1 according to the present invention was prepared.

#### EXAMPLE 2-2

Example 2-1 was repeated except that polyethylene glycol used in the overcoat layer forming liquid No. 2-1 was replaced with polyethylene glycol monocarboxylic acid ester (Trademark "Ionet MS400" made by Sanyo Chemical Industries, Ltd.), whereby a photoconductor No. 2-2 according to the present invention was prepared.

#### EXAMPLE 2-3

Example 2-1 was repeated except that polyethylene glycol used in the overcoat layer forming liquid No. 2-1 was replaced with polyethylene glycol monoether (Trademark "Emulmin L380" made by Sanyo Chemical Industries, Ltd.), whereby a photoconductor No. 2-3 according to the present invention was prepared.

#### COMPARATIVE EXAMPLE 2-1

Example 2-1 was repeated except that polyethylene glycol was eliminated from the overcoat layer forming liquid No. 2-1, whereby a comparative photoconductor No. 2-1 was prepared.

#### EXAMPLE 2-4

Example 2-1 was repeated except that the pigment No.1 used in the charge generation layer forming liquid No. 2-1 was replaced with the pigment No. 47, whereby a photoconductor No. 2-4 according to the present invention was prepared.

#### EXAMPLE 2-5

Example 2-2 was repeated except that the pigment No.1 used in the charge generation layer forming liquid employed in Example 2-2 was replaced with the pigment No. 47, whereby a photoconductor No. 2-5 according to the present invention was prepared.

#### EXAMPLE 2-6

Example 2-3 was repeated except that the pigment No.1 used in the charge generation layer forming liquid employed in Example 2-3 was replaced with the pigment No. 47, whereby a photoconductor No. 2-6 according to the present invention was prepared.

#### EXAMPLE 2-7

Example 2-1 was repeated except that polyethylene glycol used in the overcoat layer forming liquid No. 2-1 was replaced with polypropylene glycol (made by Wako Pure Chemical Industries, Ltd.), whereby a photoconductor No. 2-7 according to the present invention was prepared.

#### EXAMPLE 2-8

Example 2-2 was repeated except that polyethylene glycol monocarboxylic acid ester used in the overcoat layer forming liquid prepared in Example 2-2 was replaced with polyethylene glycol dicarboxylic acid ester (Trademark "Ionet DL200" made by Sanyo Chemical Industries, Ltd.), whereby a photoconductor No. 2-8 according to the present invention was prepared.

#### EXAMPLE 2-9

Example 2-3 was repeated except that polyethylene glycol monoether used in the overcoat layer forming liquid prepared in Example 2-3 was replaced with polypropylene glycol monoether (Trademark "Newpol LB1800X" made by Sanyo Chemical Industries, Ltd.), whereby a photoconductor No. 2-9 according to the present invention was prepared.

#### EXAMPLE 2-10

Example 2-1 was repeated except that an intermediate layer having a thickness of 0.1  $\mu\text{m}$  was interposed between the charge generation layer and the overcoat layer, whereby a photoconductor No. 2-10 according to the present invention was prepared.

The intermediate layer was formed in the following manner. An intermediate layer forming liquid was prepared by dispersing 2 parts by weight of nylon resin (Trademark "CM8000" made by Toray Industries, Inc.) in 60 parts by weight of methanol and 38 parts by weight of butanol. The resulting liquid was dip-coated onto the charge generation layer at a pulling up speed of 3 mm/sec, and then dried at 120° C. for 20 minutes, thereby forming an intermediate layer on the charge generation layer.

#### EXAMPLE 2-11

Example 2-2 was repeated except that an intermediate layer having a thickness of 0.1  $\mu\text{m}$  was interposed between the charge generation layer and the overcoat layer in the same manner as in Example 2-10, whereby a photoconductor No. 2-11 according to the present invention was prepared.

## EXAMPLE 2-12

Example 2-3 was repeated except that an intermediate layer having a thickness of 0.1  $\mu\text{m}$  was interposed between the charge generation layer and the overcoat layer in the same manner as in Example 2-10, whereby a photoconductor No. 2-12 according to the present invention was prepared.

## 2-13

Example 2-1 was repeated except that the overcoat layer forming liquid No. 2-1 was replaced with an overcoat layer forming liquid prepared in the following manner, whereby a photoconductor No. 2-13 according to the present invention was prepared.

## Preparation of Overcoat Layer Forming Liquid

The following components were dispersed in a ball mill for 72 hours, and the resulting dispersion was diluted with cyclohexanone, thereby obtaining a dispersion containing 10 wt.% of the solid components.

To this dispersion, 5 parts by weight of polybutylene glycol (Trademark "Terathane 2900" made by Du Pont Japan Ltd.) was added under stirring, whereby an overcoat layer forming liquid was prepared.

## EXAMPLE 2-14

Example 2-13 was repeated except that polybutylene glycol used in the overcoat layer forming liquid prepared in Example 2-13 was replaced with polyoxyethylene sorbitan monolaurate (Trademark "Ionent T-20C" made by Sanyo Chemical Industries, Ltd.), whereby a photoconductor No. 2-14 according to the present invention was prepared.

## EXAMPLE 2-15

Example 2-13 was repeated except that polybutylene glycol used in the overcoat layer forming liquid prepared in Example 2-13 was replaced with polyoxyethylene glycol monoether (Trademark "Emulmin L380" made by Sanyo Chemical Industries, Ltd.), whereby a photoconductor No. 2-15 according to the present invention was prepared.

## COMPARATIVE EXAMPLE 2-2

Example 2-10 was repeated except that polyethylene glycol was eliminated from the overcoat layer forming liquid prepared in Example 2-10, whereby a comparative photoconductor No. 2-2 was prepared.

The electrophotographic properties of the above-prepared electrophotographic photoconductors Nos. 2-1 through 2-15 according to the present invention and the comparative ones Nos. 2-1 and 2-2 were each evaluated using an electrostatic paper analyzer (Trademark "SP-428", made by Kawaguchi Electro Works) in the following manner.

Each of the above electrophotographic photoconductors was positively charged in the dark under application of +6 kV of corona charge for 20 seconds. The surface potential of the photoconductor  $V_2$ , 2 seconds after the initiation of the charging, was measured by the paper analyzer. The photoconductor was then allowed to stand in the dark without applying any charge thereto until its surface potential reached +800 V. The photoconductor was then illuminated by a tungsten lamp in such a manner that the illuminance on the illuminated surface of the photoconductor was 4.5 lux, so

## 50

that the exposure  $S$  (lux-sec) required to reduce the surface potential (+800 V) to +400 V was measured.

The photoconductor was then exposed to a tungsten light having a color temperature of 2856° K with an exposure of 100,000 lux-sec, and the surface potential  $V_2'$  and the exposure  $S'$  were measured again in the same manner as mentioned above.

The results are shown in Table 2-1.

TABLE 2-1

| Photo-conductor | Before Fatigue |                 | After Fatigue |                  |
|-----------------|----------------|-----------------|---------------|------------------|
|                 | $V_2$ (V)      | $S$ (lux · sec) | $V_2'$ (V)    | $S'$ (lux · sec) |
| No. 2-1         | 875            | 0.53            | 860           | 0.48             |
| No. 2-2         | 857            | 0.42            | 814           | 0.40             |
| No. 2-3         | 865            | 0.53            | 840           | 0.52             |
| No. 2-4         | 835            | 0.53            | 811           | 0.50             |
| No. 2-5         | 810            | 0.55            | 808           | 0.53             |
| No. 2-6         | 870            | 0.54            | 852           | 0.48             |
| No. 2-7         | 850            | 0.40            | 810           | 0.39             |
| No. 2-8         | 862            | 0.54            | 853           | 0.55             |
| No. 2-9         | 820            | 0.52            | 804           | 0.49             |
| No. 2-10        | 830            | 0.55            | 815           | 0.53             |
| No. 2-11        | 880            | 0.56            | 857           | 0.49             |
| No. 2-12        | 845            | 0.40            | 810           | 0.38             |
| No. 2-13        | 870            | 0.53            | 854           | 0.55             |
| No. 2-14        | 821            | 0.53            | 804           | 0.45             |
| No. 2-15        | 825            | 0.55            | 815           | 0.52             |
| Comp.           | 872            | 0.55            | 615           | 0.50             |
| No. 2-1         |                |                 |               |                  |
| Comp.           | 779            | 0.49            | 393           | 0.43             |
| No. 2-2         |                |                 |               |                  |

30 The photoconductor was attached to the surface of an Al drum having a thickness of 3 mm and a size of 80φ × 340 mm. This was placed in a copying machine (Trademark "FT 4060" made by Ricoh Company Ltd.), and images were repeatedly printed. The images were usually observed at the outset of printing and after 10,000 prints had been made. The results are shown in Table 2-2.

TABLE 2-2

| Photo-conductor | Printed Images at Outset of Printing |                             | Printed Images after 10,000-time Printing |
|-----------------|--------------------------------------|-----------------------------|-------------------------------------------|
|                 |                                      |                             |                                           |
| No. 2-1         | clear                                | clear                       |                                           |
| No. 2-2         | clear                                | clear                       |                                           |
| No. 2-3         | clear                                | clear                       |                                           |
| No. 2-4         | clear                                | clear                       |                                           |
| No. 2-5         | clear                                | clear                       |                                           |
| No. 2-6         | clear                                | clear                       |                                           |
| No. 2-7         | clear                                | clear                       |                                           |
| No. 2-8         | clear                                | clear                       |                                           |
| No. 2-9         | clear                                | clear                       |                                           |
| No. 2-10        | clear                                | clear                       |                                           |
| No. 2-11        | clear                                | clear                       |                                           |
| No. 2-12        | clear                                | clear                       |                                           |
| No. 2-13        | clear                                | clear                       |                                           |
| No. 2-14        | clear                                | clear                       |                                           |
| No. 2-15        | clear                                | clear                       |                                           |
| Comp.           | clear                                | Image density was found low |                                           |
| No. 2-1         | clear                                | Image density was found low |                                           |
| Comp.           | clear                                | Image density was found low |                                           |
| No. 2-2         |                                      |                             |                                           |

60 The results of the above tests demonstrate that the electrophotographic photoconductors according to the present invention, which comprise an overcoat layer containing the polyethylene glycol, have high sensitivity, and show extremely small reduction in the chargeability caused by pre-exposure fatigue. Furthermore, the photoconductors of the present invention bring about no delay in the rise of the charged potential and a minimized change in the residual electric potential even after repeated charging and exposing.

## EXAMPLE 3-1

## Preparation of Charge Transport Layer Forming Liquid

A charge transport layer forming liquid No. 3-1 having the following formulation was prepared.

|                                                                                      | parts by weight |
|--------------------------------------------------------------------------------------|-----------------|
| $\alpha$ -Phenylstilbene having the following formula (charge transporting material) | 10              |
|     |                 |
| Polycarbonate (Trademark "Panlite C-1400" made by Teijin Limited)                    | 10              |
| Silicone oil (Trademark "KF50", made by Shin-Etsu Silicone Co., Ltd.)                | 0.0002          |
| Tetrahydrofuran                                                                      | 80              |

## Preparation of Charge Generation Layer Forming Liquid

The azo pigment No. 1 and cyclohexanone in a weight ratio of 1:16 were placed in a ball mill pot, followed by ball-milling for 48 hours by using stainless steel balls.

Thereafter, the same amount of cyclohexanone was added to the above mixture, and ball-milling was continued for a further 24 hours.

The resulting mixture taken out of the ball mill was diluted with cyclohexanone under stirring, whereby a charge generation layer forming liquid No. 3-1 was obtained, which contained 1 wt.% of the solid components.

## Preparation of Intermediate Layer Forming Liquid

An intermediate layer forming liquid No. 3-1 having the following formulation was prepared.

|                                               | parts by weight |
|-----------------------------------------------|-----------------|
| Dicyclohexano-18-crown-6-ether                | 0.01            |
| Zirconium acetylacetone                       | 1               |
| $\gamma$ -methacryloxypropyltrimethoxy silane | 1               |
| n-Butanol                                     | 40              |

## Preparation of Protective Layer Forming Liquid

The following components were placed in a ball mill pot, followed by ball-milling for 48 hours, whereby a protective layer forming liquid No. 3-1 was prepared.

|                                                                                               | parts by weight |
|-----------------------------------------------------------------------------------------------|-----------------|
| Polyester resin (Trademark "V-200" made by Toyobo Co., Ltd.)                                  | 10              |
| Tin oxide powder containing 10 wt. % of antimony oxide (made by Mitsubishi Metal Corporation) | 10              |
| Dichloroethane                                                                                | 90              |

## Preparation of Photoconductor

An aluminum substrate was dip-coated with the above-prepared charge transport layer forming liquid at a pulling up speed of 6 mm/sec, and dried at 120° C. for 30 minutes, thereby forming a charge transport layer 2  $\mu$ m in thickness on the substrate.

Thereafter, the charge generation layer forming liquid was dip-coated onto the charge transport layer at a pulling up speed of 5 mm/sec, and dried at 120° C. for 20 minutes, thereby forming a charge generation layer on the charge transport layer.

The intermediate layer forming liquid was dip-coated onto the above-formed charge generation layer at a pulling up speed of 9 mm/sec, and dried at 80° C. for 120 minutes, whereby an intermediate layer having a thickness of 2000 Å was formed on the charge generation layer.

Finally, the protective layer forming liquid was spray-coated onto the above intermediate layer, and heated at 130° C. for 30 minutes, thereby forming a protective layer 5  $\mu$ m in thickness on the intermediate layer.

Thus, a photoconductor No. 3-1 according to the present invention was prepared.

## COMPARATIVE EXAMPLE 3-1

Example 3-1 was repeated except that dicyclohexano-18-crown-6-ether was eliminated from the intermediate forming liquid No. 3-1, whereby a comparative photoconductor No. 3-1 was prepared.

## EXAMPLE 3-2

Example 3-1 was repeated except that the pigment No. 1 used in the charge generation layer forming liquid No. 3-1 was replaced with the pigment No. 47, whereby a photoconductor No. 3-2 according to the present invention was prepared.

## COMPARATIVE EXAMPLE 3-2

Example 3-2 was repeated except that dicyclohexano-18-crown-6-ether was eliminated from the intermediate layer forming liquid No. 3-1, whereby a comparative photoconductor No. 3-2 was prepared.

## EXAMPLE 3-3

Example 3-1 was repeated except that dicyclohexano-18-crown-6-ether used in the intermediate layer forming liquid No. 3-1 was replaced with polydibenz-18-crown ether, whereby a photoconductor No. 3-3 according to the present invention was prepared.

## EXAMPLE 3-4

Example 3-1 was repeated except that the protective layer forming liquid No. 3-1 was replaced with a protective layer forming liquid prepared in the following

manner, whereby a photoconductor No. 3-4 according to the present invention was prepared.

#### Preparation of Protective Layer Forming Liquid

The following components were dispersed in a ball mill for 72 hours, and the resulting dispersion was diluted with cyclohexanone, thereby obtaining a protective layer forming liquid containing 10 wt.% of the solid components.

| parts by weight                                                                            |    |
|--------------------------------------------------------------------------------------------|----|
| 20% Cyclohexanone solution of phenoxy resin "PKHJ" (Trademark) made by Union Carbide Corp. | 25 |
| Tin oxide powder                                                                           | 5  |
| Cyclohexanone                                                                              | 70 |

#### COMPARATIVE EXAMPLE 3-3

Example 3-4 was repeated except that dicyclohexano-18-crown-6-ether was eliminated from the intermediate layer forming liquid used in Example 3-4, whereby a comparative photoconductor No. 3-3 was prepared.

#### EXAMPLE 3-5

Example 3-4 was repeated except that the intermediate layer forming liquid used in Example 3-4 was replaced with an intermediate layer forming liquid having the following formulation, whereby a photoconductor No. 3-5 according to the present invention was prepared.

#### Formulation of Intermediate Layer Forming Liquid

| parts by weight                                                 |      |
|-----------------------------------------------------------------|------|
| Nylon resin (Trademark "CM8000" made by Toray Industries, Inc.) | 2    |
| Dicyclohexano-18-crown-6-ether                                  | 0.02 |
| Methanol                                                        | 60   |
| Butanol                                                         | 38   |

#### COMPARATIVE EXAMPLE 3-4

Example 3-5 was repeated except that dicyclohexano-18-crown-6-ether was eliminated from the intermediate layer forming liquid used in Example 3-5, whereby a comparative photoconductor No. 3-4 was prepared.

The electrophotographic properties of the above-prepared electrophotographic photoconductors Nos. 3-1 through 3-5 according to the present invention and the comparative ones Nos. 3-1 and 3-4 were each evaluated using an electrostatic paper analyzer (Trademark "SP-428", made by Kawaguchi Electro Works) in the following manner.

Each of the above electrophotographic photoconductors was positively charged in the dark under application of +6 kV of corona charge for 20 seconds. The surface potential of the photoconductor  $V_2$ , 2 seconds after the initiation of the charging, was measured by the paper analyzer. The photoconductor was then allowed to stand in the dark without applying any charge thereto until its surface potential reached +800 V. The photoconductor was then illuminated by a tungsten lamp in such a manner that the illuminance on the illu-

minated surface of the photoconductor was 4.5 lux, so that the exposure  $S$  (lux-sec) required to reduce the surface potential (+800 V) to +400 V was measured.

The photoconductor was then exposed to a tungsten light having a color temperature of 1856° K with an exposure of 100,000 lux-sec, and the surface potential  $V_2'$  and the exposure  $S'$  were measured again in the same manner as mentioned above. The results are shown in Table 3-1.

TABLE 3-1

| Photo-conductor | Before Fatigue |                 | After Fatigue |                  |
|-----------------|----------------|-----------------|---------------|------------------|
|                 | $V_2$ (V)      | $S$ (lux · sec) | $V_2'$ (V)    | $S'$ (lux · sec) |
| No. 3-1         | 761            | 0.82            | 708           | 0.83             |
| No. 3-2         | 773            | 0.76            | 720           | 0.76             |
| No. 3-3         | 670            | 0.85            | 609           | 0.82             |
| No. 3-4         | 762            | 0.80            | 719           | 0.81             |
| No. 3-5         | 782            | 0.82            | 728           | 0.81             |
| Comp.           | 728            | 0.81            | 385           | 0.79             |
| No. 3-1         |                |                 |               |                  |
| Comp.           | 740            | 0.75            | 347           | 0.73             |
| No. 3-2         |                |                 |               |                  |
| Comp.           | 729            | 0.80            | 436           | 0.75             |
| No. 3-3         |                |                 |               |                  |
| Comp.           | 651            | 0.89            | 358           | 0.89             |
| No. 3-4         |                |                 |               |                  |

The photoconductor was attached to the surface of an Al drum having a thickness of 3 mm and a size of 80φ × 340 mm. This was placed in a copying machine (Trademark "FT 4060" made by Ricoh Company Ltd.), and images were repeatedly printed. The images were usually observed at the outset of printing and after 10,000 prints had been made. The results are shown in Table 3-2.

TABLE 3-2

| Photo-conductor | Printed Images at Outset of Printing |                             | Printed Images after 10,000-time Printing |
|-----------------|--------------------------------------|-----------------------------|-------------------------------------------|
|                 |                                      |                             |                                           |
| No. 3-1         | clear                                | clear                       |                                           |
| No. 3-2         | clear                                | clear                       |                                           |
| No. 3-3         | clear                                | clear                       |                                           |
| No. 3-4         | clear                                | clear                       |                                           |
| No. 3-5         | clear                                | clear                       |                                           |
| Comp.           | clear                                | Image density was found low |                                           |
| No. 3-1         |                                      |                             |                                           |
| Comp.           | clear                                | Image density was found low |                                           |
| No. 3-2         |                                      |                             |                                           |
| Comp.           | clear                                | Image density was found low |                                           |
| No. 3-3         |                                      |                             |                                           |
| Comp.           | clear                                | Image density was found low |                                           |
| No. 3-4         |                                      |                             |                                           |

The results of the above tests demonstrate that the electrophotographic photoconductors according to the present invention, which comprise an intermediate layer containing the crown ether, have high sensitivity, and show extremely small reduction in the chargeability caused by pre-exposure fatigue. Furthermore, the photoconductors of the present invention bring about no delay in the rise of the charged potential and a minimized change in the residual electric potential even after repeated charging and exposing.

#### EXAMPLE 4-1

#### Preparation of Charge Transport Layer Forming Liquid

A charge transport layer forming liquid No. 4-1 having the following formulation was prepared.

-continued

|                                                                                      | parts by weight |
|--------------------------------------------------------------------------------------|-----------------|
| $\alpha$ -Phenylstilbene having the following formula (charge transporting material) | 10              |
|     |                 |
| Polycarbonate (Trademark "Panlite C-1400" made by Teijin Limited)                    | 10              |
| Silicone oil (Trademark "KF50", made by Shin-Estu Silicone Co., Ltd.)                | 0.0002          |
| Tetrahydrofuran                                                                      | 80              |

#### Preparation of Charge Generation Layer Forming Liquid

The azo pigment No. 1 and cyclohexanone in a weight ratio of 1:16 were placed in a ball mill pot, followed by ball-milling for 48 hours by using stainless steel balls.

Thereafter, the same amount of cyclohexanone was added to the above mixture, and ball-milling was continued for a further 24 hours.

The resulting mixture taken out of the ball mill was diluted with cyclohexanone under stirring, whereby a charge generation layer forming liquid No. 4-1 was obtained, which contained 1 wt.% of the solid components.

#### Preparation of Intermediate Layer Forming Liquid

An intermediate layer forming liquid No. 4-1 having the following formulation was prepared.

|                                                                                                                            | parts by weight |
|----------------------------------------------------------------------------------------------------------------------------|-----------------|
| Polyethylene polyoxypropylene glycol (Trademark "Newpol PE68", a block copolymer, made by Sanyo Chemical Industries, Ltd.) | 0.01            |
| Zirconium acetylacetone                                                                                                    | 1               |
| $\gamma$ -methacryloxypropyltrimethoxy silane                                                                              | 1               |
| n-Butanol                                                                                                                  | 40              |

#### Preparation of Protective Layer Forming Liquid

The following components were placed in a ball mill pot, followed by ball-milling for 48 hours, whereby a protective layer forming liquid No. 4-1 was prepared.

|                                                              | parts by weight |
|--------------------------------------------------------------|-----------------|
| Polyester resin (Trademark "V-200" made by Toyobo Co., Ltd.) | 10              |
| Tin oxide powder containing 10 wt. % of antimony oxide       | 10              |

|                                                       | parts by weight |
|-------------------------------------------------------|-----------------|
| (made by Mitsubishi Metal Corporation) Dichloroethane | 90              |

#### Preparation of Photoconductor

- 10 An aluminum substrate was dip-coated with the above-prepared charge transport layer forming liquid at a pulling up speed of 6 mm/sec, and dried at 120° C. for 30 minutes, thereby forming a charge transport layer on the substrate.
- 15 Thereafter, the charge generation layer forming liquid was dip-coated onto the charge transport layer at a pulling up speed of 5 mm/sec, and dried at 120° C. for 20 minutes, thereby forming a charge generation layer on the charge transport layer.
- 20 The intermediate layer forming liquid was dip-coated onto the above-formed charge generation layer at a pulling up speed of 9 mm/sec, and dried at 80° C. for 120 minutes, whereby an intermediate layer having a thickness of 2000 Å was formed on the charge generation layer.

Finally, the protective layer forming liquid was spray-coated onto the above intermediate layer, and heated at 130° C. for 30 minutes, thereby forming a protective layer 5  $\mu$ m in thickness on the intermediate layer.

Thus, a photoconductor No. 4-1 according to the present invention was prepared.

#### EXAMPLE 4-2

- 35 Example 4-1 was repeated except that polyethylene polyoxypropylene glycol used in the intermediate layer forming liquid No. 4-1 was replaced with polyethylene glycol monocarboxylate (Trademark "Ionet MS1000" made by Sanyo Chemical Industries, Ltd.), whereby a photoconductor No. 4-2 according to the present invention was prepared.

#### EXAMPLE 4-3

- 45 Example 4-1 was repeated except that polyethylene polyoxypropylene glycol used in the intermediate layer forming liquid No. 4-1 was replaced with polypropylene glycol monoether (Trademark "Newpol LB65" made by Sanyo Chemical Industries, Ltd.), whereby a photoconductor No. 4-3 according to the present invention was prepared.

#### COMPARATIVE EXAMPLE 4-1

Example 4-1 was repeated except that polyethylene polyoxypropylene glycol was eliminated from the intermediate layer forming liquid No. 4-1, whereby a comparative photoconductor No. 4-1 was prepared.

#### EXAMPLE 4-4

Example 4-1 was repeated except that the pigment No. 1 used in the charge generation layer forming liquid No. 4-1 was replaced with the pigment No. 47, whereby a photoconductor No. 4-4 according to the present invention was prepared.

#### COMPARATIVE EXAMPLE 4-2

Example 4-4 was repeated except that polyethylene polyoxypropylene glycol was eliminated from the intermediate layer forming liquid employed in Example

4—4, whereby a comparative photoconductor No. 4—2 was prepared.

#### EXAMPLE 4—5

Example 4—2 was repeated except that the pigment No. 1 used in the charge generation layer forming liquid employed in Example 4—2 was replaced with the pigment No. 47, whereby a photoconductor No. 4—5 according to the present invention was prepared.

#### EXAMPLE 4—6

Example 4—3 was repeated except that the pigment No. 1 used in the charge generation layer forming liquid employed in Example 4—3 was replaced with the pigment No. 47, whereby a photoconductor No. 4—6 according to the present invention was prepared.

#### EXAMPLE 4—7

Example 4—1 was repeated except that polyethylene polyoxypropylene glycol used in the intermediate layer forming liquid No. 4—1 was replaced with polyoxyethylene polyoxypropylene glycol (Trademark "Newpol 75H 90000", a random copolymer, made by Sanyo Chemical Industries, Ltd.), whereby a photoconductor No. 4—7 according to the present invention was prepared.

#### EXAMPLE 4—8

Example 4—2 was repeated except that polyethylene glycol monocarboxylate used in the intermediate layer forming liquid employed in Example 4—2 was replaced with polyoxyethylene sorbitan monooleate (Trademark "Ionet T-80C" made by Sanyo Chemical Industries, Ltd.), whereby a photoconductor No. 4—8 according to the present invention was prepared.

#### EXAMPLE 4—9

Example 4—3 was repeated except that polypropylene glycol monoether used in the intermediate layer forming liquid employed in Example 4—3 was replaced with polyoxyethylene polyoxypropylene glycol monoether (Trademark "Newpol 50HB-100" made by Sanyo Chemical Industries, Ltd.), whereby a photoconductor No. 4—9 according to the present invention was prepared.

#### EXAMPLE 4—10

Example 4—1 was repeated except that the protective layer forming liquid No. 4—1 was replaced with a protective layer forming liquid prepared in the following manner, whereby a photoconductor No. 4—10 according to the present invention was prepared.

##### Preparation of Protective Layer Forming Liquid

The following components were dispersed in a ball mill pot for 72 hours, and the resulting dispersion was diluted with cyclohexanone, thereby obtaining a protective layer forming liquid containing 10 wt.% of the solid components.

| parts by weight                                                                          |    |
|------------------------------------------------------------------------------------------|----|
| 20% Cyclohexane solution of phenoxy resin "PKHJ" (Trademark) made by Union Carbide Corp. | 25 |
| Tin oxide powder                                                                         | 5  |
| Cyclohexanone                                                                            | 70 |

#### EXAMPLE 4—11

Example 4—2 was repeated except that the protective layer forming liquid employed in Example 4—2 was replaced with a protective layer forming liquid prepared in the following manner, whereby a photoconductor No. 4—11 according to the present invention was prepared.

##### 10 Preparation of Protective Layer Forming Liquid

The following components were dispersed in a ball mill for 72 hours, and the resulting dispersion was diluted with cyclohexanone, thereby obtaining a protective layer forming liquid containing 10 wt.% of the solid components.

| parts by weight                                                                          |    |
|------------------------------------------------------------------------------------------|----|
| 20% Cyclohexane solution of phenoxy resin "PKHJ" (Trademark) made by Union Carbide Corp. | 25 |
| Tin oxide powder                                                                         | 5  |
| Cyclohexanone                                                                            | 70 |

#### EXAMPLE 4—12

Example 4—3 was repeated except that the protective layer forming liquid employed in Example 4—3 was replaced with a protective layer forming liquid prepared in the following manner, whereby a photoconductor No. 4—12 according to the present invention was prepared.

##### Preparation of Protective Layer Forming Liquid

The following components were dispersed in a ball mill for 72 hours, and the resulting dispersion was diluted with cyclohexanone, thereby obtaining a protective layer forming liquid containing 10 wt.% of the solid components.

| parts by weight                                                                          |    |
|------------------------------------------------------------------------------------------|----|
| 20% Cyclohexane solution of phenoxy resin "PKHJ" (Trademark) made by Union Carbide Corp. | 25 |
| Tin oxide powder                                                                         | 5  |
| Cyclohexanone                                                                            | 70 |

#### COMPARATIVE EXAMPLE 4—3

Example 4—4 was repeated except that polyethylene polyoxypropylene glycol was eliminated from the intermediate layer forming liquid employed in Example 4—4, whereby a comparative photoconductor No. 4—3 was prepared.

#### EXAMPLE 4—13

Example 4—10 was repeated except that the intermediate layer forming liquid employed in Example 4—10 was replaced with an intermediate layer forming liquid having the following formulation, whereby a photoconductor No. 4—13 according to the present invention was prepared.

##### Formulation of Intermediate Layer Forming Liquid

| parts by weight |   |
|-----------------|---|
| Nylon resin     | 2 |

-continued

| parts by weight                                                                             |      |
|---------------------------------------------------------------------------------------------|------|
| (Trademark "CM8000" made by<br>Toray Industries, Inc.)                                      |      |
| Polyethylene polyoxypropylene<br>glycol                                                     | 0.02 |
| (Trademark "Newpol PE68", a block<br>copolymer, made by Sanyo Chemical<br>Industries, Ltd.) |      |
| Methanol                                                                                    | 60   |
| Butanol                                                                                     | 38   |

## EXAMPLE 4-14

Example 4-11 was repeated except that the intermediate layer forming liquid employed in Example 4-11 was replaced with an intermediate layer forming liquid having the following formulation, whereby a photoconductor No. 4-14 according to the present invention was prepared.

## Formulation of Intermediate Layer Forming Liquid

| parts by weight                                                       |      |
|-----------------------------------------------------------------------|------|
| Nylon resin                                                           | 2    |
| (Trademark "CM8000" made by<br>Toray Industries, Inc.)                |      |
| Polyethylene polyoxypropylene<br>glycol                               | 0.02 |
| (Trademark "Ionet MS1000" made by<br>Sanyo Chemical Industries, Ltd.) |      |
| Methanol                                                              | 60   |
| Butanol                                                               | 38   |

## EXAMPLE 4-15

Example 4-12 was repeated except that the intermediate layer forming liquid employed in Example 4-12 was replaced with an intermediate layer forming liquid having the following formulation, whereby a photoconductor No. 4-15 according to the present invention was prepared.

## Formulation of Intermediate Layer Forming Liquid

| parts by weight                                                      |      |
|----------------------------------------------------------------------|------|
| Nylon resin                                                          | 2    |
| (Trademark "CM8000" made by<br>Toray Industries, Inc.)               |      |
| Propylene glycol monoether                                           | 0.02 |
| (Trademark "Newpol LB63" made by<br>Sanyo Chemical Industries, Ltd.) |      |
| Methanol                                                             | 60   |
| Butanol                                                              | 38   |

## COMPARATIVE EXAMPLE 4-4

Example 4-13 was repeated except that polyethylene polyoxypropylene glycol was eliminated from the intermediate layer forming liquid prepared in Example 4-13, whereby a comparative photoconductor No. 4-4 was prepared.

The electrophotographic properties of the above-prepared electrophotographic photoconductors Nos. 4-1 through 4-15 according to the present invention and the comparative ones Nos. 4-1 and 4-4 were each evaluated using an electrostatic paper analyzer (Trademark "SP-428", made by Kawaguchi Electro Works) in the following manner.

Each of the above electrophotographic photoconductors was positively charged in the dark under application of +6 kV of corona charge for 20 seconds. The surface potential of the photoconductor  $V_2$ , 2 seconds after the initiation of the charging, was measured by the paper analyzer. The photoconductor was then allowed to stand in the dark without applying any charge thereto until its surface potential reached +800 V. The photoconductor was then illuminated by a tungsten lamp in such a manner that the illuminance on the illuminated surface of the photoconductor was 4.5 lux, so that the exposure  $S$  (lux-sec) required to reduce the surface potential (+800 V) to +400 V was measured.

The photoconductor was then exposed to a tungsten light having a color temperature of 2856° K with an exposure of 100,000 lux-sec, and the surface potential  $V_2'$  and the exposure  $S'$  were measured again in the same manner as mentioned above.

The results are shown in Table 4-1.

TABLE 4-1

| Photo-conductor | Before Fatigue |                 | After Fatigue |                  |
|-----------------|----------------|-----------------|---------------|------------------|
|                 | $V_2$ (V)      | $S$ (lux · sec) | $V_2'$ (V)    | $S'$ (lux · sec) |
| No. 4-1         | 781            | 0.81            | 788           | 0.83             |
| No. 4-2         | 821            | 0.81            | 830           | 0.82             |
| No. 4-3         | 771            | 0.82            | 736           | 0.81             |
| No. 4-4         | 793            | 0.75            | 800           | 0.76             |
| No. 4-5         | 833            | 0.75            | 842           | 0.76             |
| No. 4-6         | 761            | 0.85            | 725           | 0.83             |
| No. 4-7         | 693            | 0.85            | 647           | 0.82             |
| No. 4-8         | 821            | 0.86            | 806           | 0.82             |
| No. 4-9         | 761            | 0.85            | 725           | 0.83             |
| No. 4-10        | 782            | 0.80            | 789           | 0.82             |
| No. 4-11        | 822            | 0.80            | 831           | 0.80             |
| No. 4-12        | 772            | 0.81            | 739           | 0.81             |
| No. 4-13        | 802            | 0.79            | 808           | 0.81             |
| No. 4-14        | 842            | 0.79            | 851           | 0.80             |
| No. 4-15        | 792            | 0.79            | 757           | 0.77             |
| Comp.           | 728            | 0.81            | 385           | 0.79             |
| No. 4-1         |                |                 |               |                  |
| Comp.           | 740            | 0.75            | 347           | 0.73             |
| No. 4-2         |                |                 |               |                  |
| Comp.           | 729            | 0.80            | 436           | 0.75             |
| No. 4-3         |                |                 |               |                  |
| Comp.           | 651            | 0.89            | 358           | 0.89             |
| No. 4-4         |                |                 |               |                  |

The photoconductor was attached to the surface of an Al drum having a thickness of 3 mm and a size of  $80\phi \times 340$  mm. This was placed in a copying machine (Trademark "FT 4060" made by Ricoh Company Ltd.), and images were repeatedly printed. The images were usually observed at the outset of printing and after 10,000 prints had been made. The results are shown in Table 4-2.

TABLE 4-2

| Photo-conductor | Printed Images at<br>Outset of Printing |       | Printed Images after<br>10,000-time Printing |
|-----------------|-----------------------------------------|-------|----------------------------------------------|
|                 | clear                                   | clear |                                              |
| No. 4-1         | clear                                   | clear | clear                                        |
| No. 4-2         | clear                                   | clear | clear                                        |
| No. 4-3         | clear                                   | clear | clear                                        |
| No. 4-4         | clear                                   | clear | clear                                        |
| No. 4-5         | clear                                   | clear | clear                                        |
| No. 4-6         | clear                                   | clear | clear                                        |
| No. 4-7         | clear                                   | clear | clear                                        |
| No. 4-8         | clear                                   | clear | clear                                        |
| No. 4-9         | clear                                   | clear | clear                                        |
| No. 4-10        | clear                                   | clear | clear                                        |
| No. 4-11        | clear                                   | clear | clear                                        |
| No. 4-12        | clear                                   | clear | clear                                        |
| No. 4-13        | clear                                   | clear | clear                                        |
| No. 4-14        | clear                                   | clear | clear                                        |
| No. 4-15        | clear                                   | clear | clear                                        |
| Comp.           | clear                                   | clear | Image density was                            |

TABLE 4-2-continued

| Photo-conductor | Printed Images at Outset of Printing | Printed Images after 10,000-time Printing |
|-----------------|--------------------------------------|-------------------------------------------|
| No. 4-1         |                                      | found low                                 |
| Comp.           | clear                                | Image density was found low               |
| No. 4-2         |                                      | Image density was found low               |
| Comp.           | clear                                | Image density was found low               |
| No. 4-3         |                                      | Image density was found low               |
| Comp.           | clear                                | Image density was found low               |
| No. 4-4         |                                      | found low                                 |

10

The results of the above tests demonstrate that the electrophotographic photoconductors according to the present invention, which comprise an intermediate layer containing the polyethylene glycol, have high 15 sensitivity, and show extremely small reduction in the chargeability caused by pre-exposure fatigue. Furthermore, the photoconductors of the present invention bring about no delay in the rise of the charged potential and a minimized change in the residual electric potential 20 even after repeated charging and exposing.

What is claimed is:

1. An electrophotographic photoconductor comprising an electroconductive support, a photoconductive layer formed on said electroconductive support, and an 25 overcoat layer formed on said photoconductive layer, wherein said overcoat layer comprises a binder resin and one component selected from the group consisting of a crown ether, a polyalkylene glycol of molecular weight 100 or greater, a polyalkylene glycol ester and a polyalkylene glycol ether of molecular weight 322 or greater.

2. The electrophotographic photoconductor as claimed in claim 1, wherein the amount of said crown ether in said overcoat layer is in the range of 0.01 to 10 parts by weight to 1 part by weight of said binder resin.

3. The electrophotographic photoconductor as claimed in claim 1, wherein the amount of said polyalkylene glycol in said overcoat layer is in the range of 0.01 to 10 parts by weight to 1 part by weight of said 40 binder resin.

4. The electrophotographic photoconductor as claimed in claim 1, wherein the amount of said polyalkylene glycol ester in said overcoat layer is in the range of 0.01 to 10 parts by weight to 1 part by weight of said binder resin.

5. The electrophotographic photoconductor as claimed in claim 1, wherein the amount of said polyalkylene glycol ether in said overcoat layer is in the range of 0.01 to 10 parts by weight to 1 part by weight of said 50 binder resin.

6. The electrophotographic photoconductor as claimed in claim 1, wherein said overcoat layer further comprises finely-divided particles of a metallic oxide.

7. The electrophotographic photoconductor as claimed in claim 6, wherein the particle size of said metallic oxide is 0.5  $\mu\text{m}$  or less.

8. The electrophotographic photoconductor as claimed in claim 6, wherein the amount of said metallic oxide is 10 to 80 wt.  $\mu\text{g}$  of the entire weight of said overcoat layer.

9. The electrophotographic photoconductor as claimed in claim 6, wherein said metallic oxide is selected from the group consisting of  $\text{SnO}_2$ ,  $\text{Sb}_2\text{O}_3$ ,  $\text{In}_2\text{O}_3$ , and  $\text{TiO}_2$ .

10. The electrophotographic photoconductor as claimed in claim 1, wherein said overcoat layer has a thickness of 1  $\mu\text{m}$  to 30  $\mu\text{m}$ .

11. The electrophotographic photoconductor as claimed in claim 1, wherein said photoconductive layer comprises a charge generation layer and a charge transport layer.

5 12. The electrophotographic photoconductor as claimed in claim 1, wherein said crown ether is selected from the group consisting of benzo-9-crown-3-ether, 12-crown-4-ether, 18-crown-6-ether, dibenzo-18-crown-6-ether, tetrabenzo-24-crown-8-ether, 15-crown-5-ether, 21-crown-7-ether, benzo-15-crown-5-ether, dibenzo-24-crown-8-ether, dicyclohexano-24-crown-8-ether, poly(dibenzo-18-crown-6-ether) and a crown ether having the following formula:



13. The electrophotographic photoconductor as claimed in claim 1, wherein said polyalkylene glycol is selected from the group consisting of polyethylene glycol, polypropylene glycol, polybutylene glycol, a random copolymer of hydroxyethylene and hydroxypropylene, and a block copolymer of hydroxyethylene and hydroxypropylene.

14. The electrophotographic photoconductor as claimed in claim 13, wherein said polyethylene glycol has a molecular weight ranging from 100 to 5,000,000.

15. The electrophotographic photoconductor as claimed in claim 13, wherein said polypropylene glycol has a molecular weight ranging from 130 to 500,000.

16. The electrophotographic photoconductor as claimed in claim 13, wherein said polybutylene glycol has a molecular weight ranging from 160 to 100,000.

17. The electrophotographic photoconductor as claimed in claim 13, wherein said random copolymer of hydroxyethylene and hydroxypropylene has a molecular weight ranging from 200 to 500,000.

18. The electrophotographic photoconductor as claimed in claim 13, wherein said block copolymer of hydroxyethylene and hydroxypropylene has a molecular weight ranging from 200 to 500,000.

19. The electrophotographic photoconductor as claimed in claim 1, wherein said polyalkylene glycol ester is selected from the group consisting of a polyethylene glycol monocarboxylic acid ester, a polyethylene glycol dicarboxylic acid ester and a carboxylic acid ester of polyoxyethylene sorbitan.

20. The electro-photographic photoconductor as claimed in claim 1, wherein said polyalkylene glycol ether is selected from the group consisting of a polyethylene glycol monoether, a polypropylene glycol monoether and a monoether of a copolymer of hydroxyethylene and hydroxypropylene.

21. The electrophotographic photoconductor as claimed in claim 20, wherein said polyethylene glycol monoether has the formula:



wherein R represents an alkyl group having 1 to 30 carbon atoms, or a phenyl group having as a substituent an alkyl group having 1 to 20 carbon atoms; and n is an integer of 2 to 1 000.

22. The electrophotographic photoconductor as claimed in claim 20, wherein said polypropylene glycol monoether has the formula:



10  
wherein R represents an alkyl group having 1 to 30 carbon atoms, or a phenyl group having as a substituent an alkyl group having 1 to 20 carbon atoms; and n is an integer of 5 to 100.

23. The electrophotographic photoconductor as claimed in claim 20, wherein said monoether of the copolymer of hydroxyethylene and hydroxypropylene has a molecular weight of 200 to 20,000.

24. The electrophotographic photoconductor as claimed in claim 1, wherein said overcoat layer comprises an intermediate layer formed on said electroconductive support, and a protective layer formed on said intermediate layer, said intermediate layer comprising a binder resin and one component selected from the group consisting of a crown ether, a polyalkylene glycol of molecular weight 100 or greater, a polyalkylene glycol ester and a polyalkylene glycol ether of molecular weight 322 or greater.

25. The electrophotographic photoconductor as claimed in claim 24, wherein the amount of said crown ether in said intermediate layer is in the range of 0.1 to 50 parts by weight to 100 parts by weight of said binder resin.

26. The electrophotographic photoconductor as claimed in claim 24, wherein the amount of said polyalkylene glycol in said intermediate layer is in the range of 0.1 to 50 parts by weight to 100 parts by weight of said binder resin.

27. The electrophotographic photoconductor as claimed in claim 24, wherein the amount of said polyalkylene glycol ester in said intermediate layer is in the range of 0.1 to 50 parts by weight to 100 parts by weight of said binder resin.

28. The electrophotographic photoconductor as claimed in claim 24, wherein the amount of said polyalkylene glycol ether in said intermediate layer is in the range of 0.1 to 50 parts by weight to 100 parts by weight of said binder resin.

29. The electrophotographic photoconductor as claimed in claim 24, wherein said protective layer further comprises finely-divided particles of a metallic oxide.

30. The electrophotographic photoconductor as claimed in claim 29, wherein the particle size of said metallic oxide is 0.5  $\mu m$  or less.

31. The electrophotographic photoconductor as claimed in claim 29, wherein the amount of said metallic oxide is 10 to 80 wt. % of the entire weight of said protective layer.

32. The electrophotographic photoconductor as claimed in claim 29, wherein said metallic oxide is selected from the group consisting of  $SnO_2$ ,  $Sb_2O_3$ ,  $In_2O_3$ , and  $TiO_2$ .

33. The electrophotographic photoconductor as claimed in claim 24, wherein said photoconductive layer comprises a charge generation layer and a charge transport layer.

34. The electrophotographic photoconductor as claimed in claim 24, wherein said crown ether is se-

lected from the group consisting of benzo-9-crown-3-ether, 12-crown-4-ether, 18-crown-6-ether, dibenzo-18-crown-6-ether, tribenzo-18-crown-6-ether, dicyclohexano-18-crown-6-ether, tetrabenzo-24-crown-8-ether, 15-crown-5-ether, 21-crown-7-ether, benzo-15-crown-5-ether, dibenzo-24-crown-8-ether, dicyclohexano-24-crown-8-ether, poly(dibenzo-18-crown-6-ether) and a crown ether having the following formula:



10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
82

65

44. The electrophotographic photoconductor as claimed in claim 42, wherein said polypropylene glycol monoether has the formula:



wherein R represents an alkyl group having 1 to 30 carbon atoms, or a phenyl group having as a substituent

66

an alkyl group having 1 to 20 carbon atoms; and n is an integer of 5 to 100.

45. The electrophotographic photoconductor as claimed in claim 24, wherein said intermediate layer has a thickness of 10  $\mu m$  or less and said protective layer has a thickness ranging from 1  $\mu m$  to 30  $\mu m$ .

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,970,131

Page 1 of 2

DATED : 11/13/90

INVENTOR(S) : Kyoshi Taniguchi, et al.

It is certified that error appears in the above-identified patent and that said Letters Patent is hereby corrected as shown below:

Column 1, line 63, "SiO<sub>2</sub> Al<sub>2</sub>O<sub>3</sub> 3 and B<sub>4</sub>C" should read

--SiO<sub>2</sub>, Al<sub>2</sub>O<sub>3</sub> and B<sub>4</sub>C--.

Column 3, line 7, "3 t 8" should read --3 to 8--.

Column 44, line 61, after "minutes" add a period ---.--

Column 45, lines 7-8, "dibenzo18-crown-6-ether" should read

--dibenzo-18-crown-6-ether--.

Column 46, line 49, before "Trademark" add a parenthesis --(--

Column 48, line 16, "EXAMPLE -7" should read --EXAMPLE 2-7--.

Column 49, line 10, "2-13" should read --EXAMPLE 2-13--.

Column 51, line 30, before "Trademark" add a parenthesis --(--

Column 51, line 67, "fallowed" should read --followed--.

Column 54, line 5, "1856°" should read --2856°--.

Column 55, line 22, before "Trademark" add a parenthesis --(--

Column 59, line 60, "4'4" should read --4-4--.

Column 61, line 60, "wt.  $\mu$ of" should read --wt. % of--.

UNITED STATES PATENT AND TRADEMARK OFFICE  
CERTIFICATE OF CORRECTION

PATENT NO. :

4,970,131  
11/13/90

Page 2 of 2

INVENTOR(S) : Kiyoshi Taniguchi, et al.

It is certified that error appears in the above-identified patent and that said Letters Patent is hereby corrected as shown below:

Column 62, line 9, after "crown-6-ether," please insert  
--tribenzo-18-crown-6-ether, dicyclohexano-18-crown-6-ether,--.

Column 62, line 57, "electro-photographic" should read  
-electrophotographic--.

Column 62, line 67, "R--O--CH<sub>2</sub>CH<sub>2</sub>O<sub>n</sub>H" should read  
--R-O-(CH<sub>2</sub>CH<sub>2</sub>O)<sub>n</sub>H--.

Column 63, line 7, "R-O-C<sub>3</sub>H<sub>6</sub>O<sub>n</sub>H" should read  
--R-O-(C<sub>3</sub>H<sub>6</sub>O)<sub>n</sub>H--.

Column 64, line 63, R-O-CH<sub>2</sub>CH<sub>2</sub>O<sub>n</sub>H" should read  
--R-O-(CH<sub>2</sub>CH<sub>2</sub>O)<sub>n</sub>H--.

Signed and Sealed this  
Sixth Day of April, 1993

Attest:

STEPHEN G. KUNIN

Attesting Officer

Acting Commissioner of Patents and Trademarks